

Aug. 25, 1942.

R. P. DELAPLACE ET AL

2,294,227

METHOD OF ELECTROLYTICALLY POLISHING STEEL

Filed Jan. 10, 1939

*Fig. 1*



*Fig. 2*



*Fig. 3*



INVENTORS:

RENE' PAUL DELAPLACE,  
CHARLES LEON BECHARD,

*Barney & Marson*

ATTORNEYS

## UNITED STATES PATENT OFFICE

2,294,227

## METHOD OF ELECTROLYTICALLY POLISHING STEEL

René Paul Delaplace, Paris, and Charles Léon Béchard, Versailles, France, assignors to Societe Brevets Aero-Mecaniques S. A., Geneva, Switzerland, a society of Switzerland

Application January 10, 1939, Serial No. 250,236  
In Belgium February 10, 1938

3 Claims. (Cl. 204—145)

The present invention relates to methods of electrolytically polishing metals or alloys, and more especially steel, which methods are of the type in which use is made, for levelling the metal striae, of an electrolysis action in a suitable bath containing said metal which constitutes the anode (anodic polishing).

The chief object of the present invention is to provide a method of this type which is better adapted to meet the requirements of practice than the methods used up to this time, and especially to improve the efficiency and rapidity of action of the method.

Another object of the invention is to provide a device for carrying out this method.

According to an important feature of the present invention, we make use, for this polishing, of a solution which while being substantially stable from the double point of view of chemical and physical phenomena, is capable of dissolving the metal in large amounts in such manner as to cause the formation, during electrolysis, of metallic salts which are but little ionized, therefore bad conductors of electricity, said salts being of the co-called "complex" type.

In particular, according to an advantageous embodiment of the present invention, we make use of a stable solution of pyrophosphoric acid.

According to another feature of the present invention, we have recourse, for making the electrolyte, to a non-aqueous solution, that is to say a solution obtained by means of a solvent which is not water, in particular an organic solvent.

Alcohol is particularly advantageous in the case where pyrophosphoric acid is used because it helps in keeping it stable.

Other features of the present invention will result from the following detailed description of some specific embodiments thereof.

Preferred embodiments of the present invention will be hereinafter described, with reference to the accompanying drawing, given merely by way of example, and in which:

Fig. 1 diagrammatically shows a device for the anodic polishing of a piece of steel (in this example a roller axis) according to the method of the present invention, said device being made according to the present invention;

Fig. 2 shows, also diagrammatically, but partly, a device of the same kind for the anodic polishing of a roller according to the process of the invention, this device being made according to the invention;

Fig. 3 is a diagrammatic view of the operation of the invention.

The invention is intended for the anodic polishing of a piece of a metal or of a metallic alloy with a view to eliminating the very minute projections which can not be removed through mechanical methods (grinding unavoidably produces striae, whereas burnishing, for instance lead burnishing, only temporarily closes these striae).

Concerning the process considered from a general point of view, it consists in utilizing electrolysis, in the known manner, in a solution in which the piece to be treated constitutes the anode.

But, concerning more particularly this solution, it is chosen in such manner that, while being sufficiently stable from the physical and chemical viewpoints, it produces, with the metal, during electrolysis, the formation of at least one salt which is but little ionized, therefore a bad conductor of electricity, this salt being of the type called, in chemistry, "complex salt."

The present invention is based upon the teaching of experience, the phenomena which take place during the electrolysis being probably those hereinafter described (it being well understood that the following explanations must be considered merely as a hypothesis):

When an anodic polishing takes place, the piece to be treated A acting as anode (Fig. 3), with striae which, on the drawing, are shown on an enlarged scale with respect to the cathode shown at C, there is a tendency to the formation, on the surface of the anode, of a layer *a* resulting from the electrolytic reactions, the layer in question having a resistance different from, and higher than, that of solution *b*.

The invention is based upon the idea that it is advantageous to increase as much as possible the resistance of this layer *a*, with a view to making as high as possible the efficiency of the electrolytic attack of the metal and to accelerate the action tending to level up the striae. This action seems to be determined by the fact that the ratio of the resistances to the flow of the current respectively opposite the projections and the hollows, that is to say:

$$\frac{r+R_1}{r+R_2}$$

in which *r* is very low in comparison with *R*<sub>1</sub> and *R*<sub>2</sub>, is but little different from:

$$\frac{R_1}{R_2}$$

the resistance being, at the beginning, very low in

comparison with  $R_2$ , it follows that there is a levelling action until  $R_1$  is equal to  $R_2$ .

Therefore our object is to accelerate this levelling and to make it more efficient, according to the invention, by increasing the resistance of layer  $a$ , and this in such manner that, owing to a suitable choice of the electrolyte, said layer tends to be constituted during the electrolytic operation, by a complex salt, that is to say a salt which is a bad conductor of electricity.

It will be readily understood that it will be easy, for someone skilled in the art, to find various embodiments of the present invention, provided that this electrolyte is:

a. On the one hand of an electrical resistance  $r$  sufficiently low;

b. Of a viscosity at least equal to that of water (averaging one centipoise), in order not to interfere with the physical stability of the active layer of the anode. However, this viscosity must not be too high so that it does not prevent the gaseous disengagements that take place on the anode and the cathode (for instance, it would be maximum at some poises, although this is but a mere indication without involving any limitation).

Among the solutions capable of producing such complex salts, and, in a more general manner, but not exclusively, according to the application of the invention which will now be considered, in the case of an anodic polishing of steel:

We may cite, for instance, oxalic acid, potassium oxalate, perchloric acid, polyphosphoric acid, and so on: it being well understood that the solution that is considered is nonaqueous, the solvent being organic and preferably alcohol.

Among the bodies above cited, the derivatives of phosphorus give particularly interesting results:

For instance, starting from a solution prepared by saturating with phosphoric anhydride a solution of ortho-phosphoric acid of 40° Bé, we found a considerable improvement of the reflecting power of the surface thus treated.

The anhydride is added as quickly as it is possible in view of the violent heating of the solution, in such manner as to obtain a viscous solution which contains a mixture of orthophosphoric, pyrophosphoric, and polyphosphoric acid.

But, as a matter of fact, the best result seems to be produced by pyrophosphoric acid, which probably produces a complex salt, such as acid pyrophosphate of iron (since iron pyrophosphate is dissolved and then combines with pyrophosphoric acid).

For instance, according to the preferred embodiment of the present invention, this pyrophosphoric acid is incorporated with a solvent such as alcohol, in such manner as to obtain a stable solution.

Advantageously, this solution will be concentrated, for instance at the rate of 400 grams of pyrophosphoric acid per liter.

The method according to the present invention being thus defined, it goes without saying that, concerning the devices or apparatus for carrying out this method it will be possible to find various embodiments in accordance, for instance, with the shape and size of the pieces to be treated.

These devices or apparatus must be arranged in such manner that they permit of rapidly evacuating the calories developed in the solution by the flow of the current. In order to obtain such a result, according to the present invention, if use is made, as diagrammatically shown by Fig. 1,

of a vessel  $1$  acting as cathode, this vessel may be made of aluminium or another metal which is a good conductor of heat.

On the other hand, concerning the electric current to be provided in these apparatus, it must flow through a circuit provided with means for feeding said current at the desired value, said means including, for instance, a rheostat  $R^h$ .

The intensity of the current to be applied at the beginning of the operation will be such that it produces a quick disengagement of oxygen on the anode. Then this intensity spontaneously rises, and the temperature, in the case of steel, averages 20° C.

Then the intensity is adjusted in such manner that it tends neither to rise nor to drop spontaneously, this value corresponding to a good working of the polishing operation. This value, in the case of the pyrophosphate solution above referred to, is about 30 amperes per square decimeter.

On the other hand, it should be noted that the polishing effect may be temporarily stopped by the phenomenon known as "passivation" of steel. This phenomenon can easily be stopped by contact with a copper rod kept in a very clean state, or by a mechanical system capable of automatically producing, from time to time, or when necessary, such a contact.

Concerning the means to be provided, in connection with this apparatus, for holding the piece to be treated, said means depend upon the shape of the piece in question.

For instance, in the case of a roller axis, as shown by Fig. 1, said piece is suspended in vessel  $1$  by means of a steel piece  $3$ , which constitutes the electrode support  $3$ , the whole being arranged in such manner that the current distribution over the surface to be polished is as uniform as possible.

In the embodiment of Fig. 2, it has been supposed that the piece to be polished consists of a roller  $4$ , the latter being, for instance placed upon an iron tripod  $5$ . The cathode can be prolonged by a rod  $6$  which is placed at the center of the roller. As to the current inlet to the anode, it can take place by mere contact of an electrode  $3$  which may pass across an external glass tube  $7$ .

It should be well understood that any other arrangements can be utilized, according to the shape and size of the pieces to be treated.

In any case, whatever be the embodiment that is adopted, it is possible, owing to the process according to the present invention, to obtain a polishing which is so perfect that no such result had been obtained up to the present time.

For instance, for an axis such as shown by Fig. 1, and when use is made of a solution of pyrophosphoric acid in alcohol, the polishing operation is performed in a period of time of about ten minutes. Then the piece is removed as rapidly as possible, and it is then immersed in an acid solution, so as to dissolve the traces of ferric pyrophosphate which may have been carried along by the surface. For this purpose, use is made, for instance, of an aqueous diluted solution of orthophosphoric acid.

The whole is then washed with distilled water and alcohol and it is then dried by means of a dry cloth.

In all cases, polishing will be produced by a kind of cleaning action exerted on the surface of the metal surface, removing all the minute projections thereof. Such a polishing is perfect

and eliminates any possibility of seizing of the pieces, while it increases their resistance.

In a general manner, while we have, in the above description, disclosed what we deem to be practical and efficient embodiments of the present invention, it should be well understood that we do not wish to be limited thereto as there might be changes made in the arrangement, disposition, and form of the parts without departing from the principle of the present invention as comprehended within the scope of the appended claims.

What we claim is:

1. A method of anodic polishing of a steel body which comprises, arranging the steel body as an 15

anode in an electrolytic bath essentially consisting of pyrophosphoric acid in non-aqueous solution in a solvent capable of assuring the stability of the acid during the course of the polishing operation, and passing an electric current through said bath.

2. In a method according to claim 1, the solvent being alcohol.

3. In a method according to claim 1, the solvent being alcohol, and the concentration of the solution being 400 g. of pyrophosphoric acid per liter.

RENÉ PAUL DELAPLACE.

CHARLES LÉON BÉCHARD.